

## UNITED STATES PATENT OFFICE.

CHARLES W. PORTER, OF BERKELEY, CALIFORNIA.

## PROCESS OF MAKING AN EXPLOSIVE SHELL.

No Drawing.

Application filed October 16, 1920. Serial No. 417,463.

*To all whom it may concern:*

Be it known that I, CHARLES W. PORTER, a citizen of the United States, and a resident of Berkeley, county of Alameda, and 5 State of California, have invented a new and useful Process of Making an Explosive Shell, of which the following is a specification.

My invention relates to a method of preparing blasting gelatin or other nitroglycerine products for use in shells, and has for 10 its object the prevention of premature explosions.

It is known that shells loaded with nitro- 15 glycerine products such as blasting gelatin, giant powder and cordite often explode while being lowered into place; such explosions usually occurring in deep wells containing water. In most instances these 20 spontaneous explosions have occurred after the shells were at depths more than 1000 feet below the water level. In dry wells such explosions occur only when the shells reach regions of high temperature.

25 As ordinarily prepared the shell consists of a tube from three to eight inches in diameter and from three to twenty feet long. The tube is filled by pressing into it a plastic preparation, known as blasting gelatin, 30 comprising nitroglycerine and other substances such as nitrocellulose, wood pulp and inorganic salts. In the preparation of the shell, no attempt is made to exclude air and more or less of it is incorporated within the 35 mass of the explosive mixture.

I conceived the idea that premature explosions might be due to the presence of air, which at high temperature, or under high pressure, causes spontaneous combustion of 40 the explosive material thereby producing, locally, sufficient heat to detonate the mass. Accordingly, I planned and carried out a number of experiments with blasting gelatin, a nitroglycerine product, mixed with 45 air under various pressures ranging from one to sixty atmospheres, and repeated the

experiments using inert gases such as carbon dioxide and nitrogen instead of air. The experiments indicate first, that blasting gelatin explodes if suddenly compressed with 50 air but is stable under the same compression with nitrogen or with carbon dioxide.

My explosive therefore comprises a nitroglycerine product in which an inert gas takes the place of the air usually incorporated in the mass. For convenience in use, I charge my explosive into a cartridge, shell or other container, and I accomplish the exclusion of the air from the container by forcing a gas such as carbon dioxide, 55 nitrogen, argon, or helium into the container before introducing the explosive material.

These inert gases are available commercial products. They are generally stored 60 and transported under pressure in steel cylinders. I convey the gas from such source by means of glass, rubber or metal tubing to the shell or cartridge and allow the gas to flow into said shell or cartridge 65 until the air originally present has been forced out and displaced by the inert gas thus introduced. Blasting gelatin or any other nitroglycerine product is then forced into the shell or cartridge in the usual way. 70 The interstices of the mass including the spaces between the separate portions of gelatin introduced into the shell are thus filled with an inert gas instead of air.

I claim:

1. The process of making an explosive shell which comprises first filling the shell with an inert gas, and then introducing the explosive.

2. The process of making an explosive 85 shell which comprises first filling the shell with carbon dioxide and then introducing a nitro-glycerine product.

In testimony whereof, I have hereunto set my hand.

CHARLES W. PORTER.